

1

3,397,970

**POUR POINT DEPRESSANT ADDITIVE**

Barney R. Strickland, Westfield, N.J., assignor to Esso Research and Engineering Company, a corporation of Delaware

No Drawing. Filed May 18, 1964, Ser. No. 368,414

2 Claims. (Cl. 44—62)

**ABSTRACT OF THE DISCLOSURE**

Middle distillate fuel containing a copolymer of ethylene and a  $C_2$  to  $C_5$  olefinically unsaturated ester pour depressant tending to promote the formation of water haze, is inhibited against said haze by a combination of the dimer of linoleic acid and quaternary ammonium salt.

The present invention is broadly concerned with a multi-purpose additive for middle distillates. The invention more particularly relates to improving the flow characteristics of middle distillates. More particularly, the invention is concerned with an additive composition which improves the flow characteristics and the haze characteristics of middle distillates. This additive composition, in essence, comprises a dimer of linoleic acid in conjunction with a quaternary ammonium salt and a copolymer of ethylene and vinyl acetate.

With the increase in the use of hydrocarbon fuels of all kinds, a serious problem has arisen in areas frequently subjected to low temperatures with respect to the cold test characteristics of fuels. Particularly, serious problems have been encountered with heating oils and diesel and jet fuels that have too high a pour point, resulting either in distributional or operating difficulties or both. For example, the distribution of heating oils by pumping or syphoning is rendered difficult or impossible at temperatures around or below the pour point of the oil. Furthermore, the flow of the oil at such temperatures from the fuel storage tank to the burner or engine cannot be maintained leading to the failure of the equipment to operate.

Also the low temperature properties of petroleum distillate fuels boiling in the range between about 250° and about 750° F. have attracted increasing attention in recent years because of the growth of market for such fuels in sub-arctic areas and because of the development of turbo-jet aircraft capable of operating at altitudes where temperatures of —50° F. or lower may be encountered.

It is, therefore, one object of the present invention to produce a pour depressant composition for middle distillates and lighter oils which will greatly enhance the quality of these fuels. In general, these oils boil in the range from about 250° to 750° F.

It is a still further object of the present invention to provide heating oils, diesel fuel oils, kerosenes and jet fuels having low pour points and having other desirable characteristics. Aviation turbo-jet fuels in which the present compositions may be used normally boil between about 250° and about 550° F. and are used in both military and civilian aircraft. Such fuels are more fully defined by U.S. Military Specifications MIL-F-5624C, MIL-F-25554A, MIL-F-25558A, and amendments thereto. Kerosenes and heating oils will normally have boiling ranges between about 300° and about 750° F. and are more fully described in ASTM Specification D-396-48T and supplements thereto, where they are referred to as No. 1 and No. 2 fuel oils. Diesel fuels in which the polymers may be employed are described in detail in ASTM Specification

2

D-975-53T and later versions of the same specification. This additive composition, in essence, comprises a dimer of linoleic acid in conjunction with a quaternary ammonium salt and a copolymer of ethylene and vinyl acetate.

5 Thus one ingredient of the compositions of the present invention are copolymers of ethylene and up to about 50% by weight of an olefinically unsaturated aliphatic monomer containing from about 3 to 5 carbon atoms per molecule. In general, these monomers may comprise vinyl acetate, vinyl propionate, methyl methacrylate, allyl ethyl ether, divinyl ether, acrylonitrile, vinylacetonitrile and the like. The preferred copolymers comprise ethylene-vinyl acetate copolymers. It is preferred that the parts by weight of ethylene in the copolymer be in the range from about 60 to 99% as compared to parts by weight of vinyl acetate in the range from about 40 to about 1%. A very desirable ethylene-vinyl acetate copolymer contains about 15 to 28% by weight of vinyl acetate, as for example about 20 parts by weight of vinyl acetate.

10 The molecular weights of the ethylene-vinyl acetate copolymer are critical and should be in the range from about 1,000 to 3,000, preferably in the range from about 1,500 to 2,200. The molecular weights are determined by K. Rast's method (Ber. 55, 1051, 3727 (1922)). These copolymers are generally described in U.S. Patent No. 3,048,479 issued Aug. 7, 1962, entitled, "Ethylene-Vinyl Ester Pour Depressant for Middle Distillates." Inventors: Stephan Ilnyckyj and Charles B. Rupar.

15 While the copolymer pour depressants as described are very effective and useful, they tend to promote formation of a water haze in the oil. Thus in accordance with one specific adaptation of the present invention, a dimer of linoleic acid is used in conjunction with a quaternary ammonium chloride in conjunction with the ethylene-vinyl acetate pour depressant. In accordance with other specific adaptations of the present invention, it is also much preferred to use other additives in conjunction with these particular compositions.

20 In order to further illustrate the invention, a dimer of linoleic acid (Santolene C) was added to a number of base fuels with the following results (normally used in fuels as a corrosion inhibitor):

TABLE I—SANTOLENE C<sup>1</sup> WITHOUT POUR DEPRESSANT INCREASES HAZE

| Base oil <sup>3</sup> | Waring blender haze test <sup>2</sup> |                                              |
|-----------------------|---------------------------------------|----------------------------------------------|
|                       | No Santolene C                        | +5 lbs. of Santolene C per 1,000 barrels oil |
| A                     | 13                                    | 27                                           |
| B                     | 4                                     | 14                                           |
| C                     | 8                                     | 12                                           |
| D                     | 13                                    | 16                                           |

50 <sup>1</sup> A solution consisting of about 45 wt. percent dimer of linoleic acid, about 5 wt. percent alkyl phosphate ester and about 50 wt. percent kerosene, so that the total additive contains about 0.40% phosphorus.

<sup>2</sup> 200 ml. oil plus 2 ml. of sea water are mixed in a Waring Blender at high speed for about 2 min., and then the mixture is centrifuged for about 10 min. The reading is made on a photoelectric colorimeter. The hazy oil is compared with the filtered sample and the reading taken in loss of percentage of light transmission (the higher the reading, the hazier the oil).

55 <sup>3</sup> All base oils contained: 75 parts per million of Primene 81R, <sup>a</sup> 10 parts per million of Aliquat 221, <sup>b</sup> 25 parts per million of HO 32. <sup>c</sup>

<sup>a</sup> In essence, a primary amine containing mainly  $C_{12}$ — $C_{14}$  tertiary alkyl groups. Prepared by reacting trisobutylene with ammonia ( $C_{12}$ — $C_{16}$ ) (normally functions as an anti-oxidant to improve sediment and color stability in storage).

<sup>b</sup> A solution of about 25 wt. percent isopropyl alcohol and water, and about 75 wt. percent of dimethyl dicoco quaternary ammonium chloride. Coco is any alkyl group from coconut oil.

<sup>c</sup> An oil solution consisting of about 25 wt. percent light mineral oil and about 75 wt. percent of tallow (stearate) fumarate/ $C_8$  oxo chloropropylene oxy maleate/vinyl acetate copolymer (sludge dis-

65

The base fuels used in these tests had boiling ranges of 325° to 660° F., API gravities of 31-33, viscosities of 34-35 SUS at 100° F. and pour points ranging from -10° to +10° F.

From the above it is apparent that the mere addition of the Santolene C further increased the haze of the composition. Additional tests were conducted wherein various amounts of the ethylene-vinyl acetate copolymer pour depressants were used in conjunction with Aliquat 221 and Santolene C with results as shown in Table II.

TABLE II.—SANTOLENE C AND ALIQUAT 221 REDUCE HAZING DUE TO POUR DEPRESSANT<sup>1</sup>

| Base oil | Copolymer pour depressant, p.p.m. | Extra <sup>2</sup> aliquat, p.p.m. | Santolene C, p.p.m. | Waring blender haze |
|----------|-----------------------------------|------------------------------------|---------------------|---------------------|
| A-----   | None                              | None                               | None                | 13                  |
|          | 250                               | None                               | None                | 92                  |
|          | 500                               | None                               | None                | 93                  |
|          | 500                               | 10                                 | None                | 36                  |
|          | 500                               | None                               | 16.5                | 89                  |
|          | 500                               | 10                                 | 16.5                | 9                   |
| E-----   | None                              | None                               | None                | 16                  |
|          | 250                               | None                               | None                | 92                  |
|          | 500                               | None                               | None                | 95                  |
|          | 500                               | 10                                 | None                | 28                  |
|          | 500                               | None                               | 16.5                | 28                  |
|          | 500                               | 10                                 | 16.5                | 4                   |

<sup>1</sup> Pour depressant was a copolymer of ethylene and vinyl acetate having 28% of vinyl acetate present and a molecular weight of about 2,000. The pour depressant was used in a solution consisting of about 50 wt. percent kerosene containing about 50 wt. percent of the copolymer. The amount of actual copolymer is half the p.p.m. shown in the table.

<sup>2</sup> Samples already contained 10 p.p.m. aliquat.

From the above it is apparent that using the copolymer pour depressant in conjunction with Santolene C (dimer of linoleic acid) and in conjunction with Aliquat 221 (quaternary ammonium salt), unexpected desirable results are secured.

Thus very desirable additive compositions to be used are the following:

TABLE III

| Additive compositions                                   | P.p.m. | Range (p.p.m.) | Range (p.p.m.) active ingredient |
|---------------------------------------------------------|--------|----------------|----------------------------------|
| Santolene C (dimer of linoleic acid)-----               | 16.5   | 2-40           | 9-18                             |
| Aliquat 221 (quaternary salt)-----                      | 20.0   | 5-30           | 3½-22.5                          |
| HO 32 (tallow fumarate)-----                            | 25.0   | 10-100         | 5-50                             |
| Primene 81 R (primary amine, etc.)-----                 | 75.0   | 5-100          | 5-100                            |
| Copolymer pour depressant (ethylene-vinyl acetate)----- | 500.00 | 100-1,000      | 50-500                           |

From the foregoing it is apparent that the haze-forming tendency of the copolymer pour depressant is materially improved by using in conjunction therewith a dimer of linoleic acid and a quaternary ammonium chloride salt.

While the foregoing is very excellent, it has also been discovered that the haze-promoting tendency of the copolymer may be controlled by adding to the base fuel in conjunction with the ethylene-vinyl acetate copolymer from about 4 to 25 p.p.m., preferably 10 to 20 p.p.m. of dicoco dimethyl ammonium nitrite. Other tests were conducted using various amounts of the copolymer in con-

junction with various amounts of Aliquat 221. The results of these tests are as follows:

TABLE IV.—ALIQUAT 221 OFFSETS HAZE STABILIZATION OF COPOLYMER

| p.p.m. <sup>3</sup> of Copolymer (ethylene-vinyl acetate) | Haze after 10 min. centrifuging, p.p.m. Aliquat 221 |       |       |       |       |       |       |       |
|-----------------------------------------------------------|-----------------------------------------------------|-------|-------|-------|-------|-------|-------|-------|
|                                                           | 0                                                   | 5     | 10    | 15    | 20    | 25    | 30    | 35    |
| 0-----                                                    | 10                                                  | 10    | 9     | 8     | 10    | 8     | 7     | ----- |
| 25-----                                                   | 32                                                  | ----- | ----- | ----- | ----- | ----- | ----- | ----- |
| 50-----                                                   | 46                                                  | 11    | 11    | 7     | 5     | ----- | ----- | ----- |
| 100-----                                                  | 55                                                  | 20    | 10    | 7     | 7     | ----- | ----- | ----- |
| 200-----                                                  | 68                                                  | 65    | 16    | ----- | 8     | 6     | 6     | 7     |
| 500-----                                                  | 62                                                  | 67    | 36    | 13    | 9     | 6     | 8     | 8     |
| 800-----                                                  | 64                                                  | 20    | 12    | 8     | 5     | 7     | 6     | 6     |

Conditions of Test.—Base oil: 70% Varsol,<sup>1</sup> 30% Primol; <sup>2</sup> viscosity: 2.6 centistokes.

<sup>1</sup> Mineral spirits—A paraffinic hydrocarbon solvent boiling in the range from about 300° to 400° F.

<sup>2</sup> An industrial white oil highly refined with fuming sulfuric acid.

<sup>3</sup> The p.p.m. are in terms of a solution of 50 wt. percent copolymer and 50 wt. percent kerosene. Actual p.p.m. of copolymer per se are half the values shown.

From the above it is apparent that when using as high as 800 parts per million of the copolymer pour depressant solution, the haze can be materially lowered by the utilization of from about 5-35 parts per million of the Aliquat 221.

Thus, the present invention is concerned with an improved middle distillate oil of improved pour characteristics and being substantially haze free. The middle distillate contains an effective amount of an ethylene-vinyl acetate copolymer pour depressant and an effective amount of a quaternary ammonium salt. Preferred middle distillate compositions contained effective amounts of an ethylene-vinyl acetate copolymer pour depressant used with effective amounts of dimers of linoleic acid and also in conjunction with a quaternary ammonium salt. Highly desirable compositions are middle distillate compositions containing an ethylene-vinyl acetate copolymer pour depressant in conjunction with a dimer of linoleic acid, in conjunction with a quaternary ammonium salt, in conjunction with a primary amine containing mainly C<sub>12</sub>-C<sub>14</sub> tertiary alkyl groups and a tallow stearate fumarate vinyl acetate copolymer.

What is claimed is:

1. A petroleum distillate oil boiling in the range of 300° to 750° F. containing a pour depressing amount of a copolymer of 60 to 99 wt. percent of ethylene and within the range of 1 to 40 wt. percent of an olefinically unsaturated C<sub>3</sub> to C<sub>5</sub> aliphatic ester monomer, said copolymer having a molecular weight of about 1,000 to 3,000 and tending to promote the formation of water haze in said oil, and as an inhibitor of said haze about .9 to 18 parts per million of dimer of linoleic acid and quaternary ammonium salt selected from the group consisting of 3½ to 22.5 p.p.m. of dicoco dimethyl ammonium chloride and 4 to 25 p.p.m. of dicoco dimethyl ammonium nitrite.

2. A composition according to claim 1, wherein said ester monomer is vinyl acetate, said salt is dicoco dimethyl ammonium chloride, and said oil has a natural pour point of -10° F. and higher.

#### References Cited

#### UNITED STATES PATENTS

|    |           |         |                       |       |
|----|-----------|---------|-----------------------|-------|
| 65 | 2,861,874 | 11/1958 | O'Kelly et al. -----  | 44-62 |
|    | 3,008,813 | 11/1961 | Siegel -----          | 44-62 |
|    | 3,048,479 | 8/1962  | Ilnyckyj et al. ----- | 44-62 |

DANIEL E. WYMAN, Primary Examiner.

Y. H. SMITH, Assistant Examiner.